

June 13, 1939.

S. KIESSKALT ET AL

2,162,200

PROCESS OF PREPARING DISPERSIONS OF COAL AND OIL

Filed May 18, 1936



Inventors:  
Siegfried Kiesskalt,  
Kurt Dampfle,  
Karl Winnacker,  
Ernst Weingartner,  
By Potter, Pease & Scheffler  
ATTORNEYS.

## UNITED STATES PATENT OFFICE

2,162,200

PROCESS OF PREPARING DISPERSIONS OF  
COAL AND OIL

Siegfried Kiesskalt, Hans Tampke, Karl Wacker, and Ernst Weingaertner, Frankfort-on-the-Main, Germany, assignors to I. G. Farbenindustrie Aktiengesellschaft, Frankfort-on-the-Main, Germany

Application May 18, 1936, Serial No. 80,440  
In Germany May 24, 1935

13 Claims. (Cl. 44—1)

The present invention relates to a process of preparing dispersions of coal and oil.

We have found that flowing coal poor in ash and in some cases even free from ash can be made in one operation in the following manner:

Coal is ground in water in any desired grinding apparatus, for instance in a tube mill or an oscillating device, and in the form of a thick viscous paste is kneaded with oil in a kneading apparatus so as to form a coherent, plastic mass. During this kneading operation the water contained in the paste of coal first separates almost completely and may be drawn off. Simultaneously a considerable portion of the ash is removed together with the water. By a subsequent washing operation during the kneading this ash removal can be enhanced. By adding the oil by degrees (in 2 to 3 portions) and simultaneously washing with water, it is possible to diminish the ash content of the paste of coal to about 0.5 per cent. During the entire operation the plastic condition of the dispersion of coal and oil is maintained.

During the grinding with water the hydrophile gangue is thoroughly broken up and wetted. During the kneading of the very viscous paste an intensive mixing of the water phase and the oil phase is produced by the shearing force of the kneading movement, and the ash together with the water is eliminated from the dispersion of coal and oil.

By the name "Trent" process there is known a process according to which coal ground in water is made into a paste with oil and an excess of water and then further treated with a relatively small quantity of oil in a flotation device. During this treatment the coal particles wetted with oil float upwards and are then drawn off in the form of a non-coherent mass. This process has the drawback that it requires disproportionately large quantities of water and, in consequence, large dressing devices. In contradistinction thereto the present process has the advantage that it is possible to obtain a complete removal of ash with a considerably smaller addition of water by the kneading with water together with oil.

The separation may be hastened and the extent of the ash removal and the desiccation may be increased by adding, according to the character of the coal and the oil, a small proportion of an acid or a base. For instance, the ash removal from, and desiccation of, lignite, with the use of lignite tar oils, may be favored by the addition of acids as, for instance, hydrochloric acid, sul-

furic acid, acetic acid, oleic acid and phenols. It may be understood, however, that lignite may be treated also with other oils by adding acids. On the other hand the ash removal from and desiccation of, coal by means of coal tar oil is considerably accelerated by the presence of a small quantity of a base, for instance, caustic soda solution, caustic potash solution and aniline. The acid or base may be added to the aqueous paste before or during the kneading or to the oil.

We have furthermore found that some kinds of lignite can yield a dispersion of coal and oil which flows well and can be conveyed with the usual pump devices by using a paste of coal and water which has been made with a coal having a content of water of not more than about 35 per cent. In this case it is immaterial whether there is used a coal in the wet state in which it comes from the mine and already containing in this state not more than about 35 per cent. of water, or a coal which has previously been dried until its water content does not exceed 35 per cent. It is surprising that the flowing power of a paste prepared with the aid of a coal of this kind is maintained even in cases in which the coal is subsequently made by addition of water into a paste of a suitable and increased content of water in order to obtain a mass capable of being kneaded.

It may be particularly advantageous to use roller mills as kneading apparatus for carrying out this process. Whereas, in general, in the treatment in roller mills pigments or filling materials are rolled into viscous, plastic masses, for instance dyestuffs into linseed oil varnish or soot into caoutchouc, it has been observed that in some cases also separating effects can be obtained in roller mills, this being surprising. In a system consisting of coal containing ash, oil and water obtained by an intensive mixing, water and ash may, for instance, be separated by treating the mixture in a roller mill. During this treatment it is noted that when the mixture enters the pass between the rollers, by the action of the shearing force of the intake movement, first the water is squeezed outwards from the mixture and then the ash constituents are eliminated with the water.

The drawing diagrammatically shows a device with a roller mill, which device is suitable for carrying out the present process. At the inlet 2 the transporting worm 1 is charged with water and finely ground coal which may be ground together in a suitable grinding apparatus. At the inlet 3 oil is added thereto. The mixture is

conveyed by the transporting worm to the rollers 4 and 5 which are very closely adjusted. In the centre above the two rollers a sump 6 is formed wherein the mixture of coal, oil and water is treated. By the rotation of the rollers the paste is moved in the direction indicated by arrows. A small quantity of the paste is continuously pressed from the sump 6 between the rollers and forms at the under ports of the rollers a thin film 7 and 8 the weight of which is about  $\frac{1}{5}$  of the mass in the sump 6. During the going through between the rollers the main quantity of the water contained in the paste is removed and drops to the bottom 9. The films 7 and 10 8 are loosened from the rollers by scrapers 10 and 11 and fall over slide plates 12 and 13 into suitable containers.

The advantage of using roller mills for this process is that on the one hand the operation 20 may be continuous with a considerably lower consumption of power than, for instance, in a Werner-Pfleiderer kneading apparatus. On the other hand, by the action of the shearing force on the highly viscous paste the particles of coal 25 are more finely crushed so that further particles of ash are dissociated from the coal and eliminated. It follows that an additional quantity of ash may thus be separated from the paste from which with the aid of kneading and watering 30 in the Werner-Pfleiderer kneading apparatus ash can no longer be separated.

The kneading process which according to the properties of the coal lasts only a few minutes 35 may be considerably accelerated by an addition which increases the tendency for the coal to be wetted by oil and reduces the tendency for it to be wetted by water, such as tetrahydronaphthalene, benzene, aniline and alcohols of high molecular weight. The separation of water 40 caused by the kneading process may be improved by the application of a temperature of about 40° C. to 100° C., and if required, by the application of a reduced pressure.

The grinding operation in the aqueous phase 45 preceding the kneading operation affords an opportunity for a simultaneous chemical treatment, such as desulfurization, removal of iron and the like.

The process may be applied for the manufacture 50 of flowing coal, and also for the manufacture of dust coal poor in ash in which case the oil, suitably of low boiling point, present in the paste is evaporated. By this method it is also possible to make dispersions of graphite in lubricating oils, such as are used for lubricating movable engine parts. For this purpose there are 55 suitable not only graphite but also anthracite, coal, lignite, coke and semi-coke, but particularly waste coal rich in ash as obtained in the washeries of the coal dressings.

In comparison with the hitherto usual method 60 for the manufacture of flowing coal, the process has, apart from the quality of the products obtained, the advantage that it is possible to apply the wet grinding process for the manufacture of flowing coal free from or poor in ash, whereby there is attained, in comparison with the dry grinding process, a considerable saving of energy with an improved output of fineness.

In comparison with the known flotation process 70 the process of the present invention is distinguished by the fact that in the plastic phases there is required only a fraction of the water which must be used in these known processes.

The following examples serve to illustrate the

invention, but they are not intended to limit it thereto: the parts are by weight:

(1) 100 parts of a waste coal slime containing 22 per cent. of ash is finely ground in a tube mill with the addition of about 100 parts of water. In known kneading machines, such as a Werner-Pfleiderer kneading apparatus, kneading worms or the like, the aqueous paste is kneaded with 100 parts of a mineral oil. After some minutes the water and most of the ash separate. A dispersion 10 of coal and oil is produced containing only 1 per cent. of ash.

(2) A coal having an ash content of 8.3 per cent. is treated as described in Example 1. The dispersion of coal and oil of 50 per cent. strength 15 which is produced shows an ash content of only 1 per cent.

(3) 100 parts of a lignite coke containing 19.2 per cent. of ash is finely ground with 100 parts of water for about 15 hours in an oscillating 20 device such as that described in U. S. patent application Serial No. 731,172, filed June 18, 1934, in the name of Siegfried Klesskalt and Walther Mejer. The aqueous paste so obtained is then kneaded in a Werner-Pfleiderer kneading apparatus with 100 parts of a mineral oil. Together with the separation of the water most of the ash separates and is eliminated by elutriation with water. There is obtained a dispersion of coke and oil containing 4.1 per cent. of ash. 30

(4) 100 parts of a dry coal having an ash content of 14.4 per cent. and 50 parts of water are made into a paste in a known kneading apparatus. After the addition of 100 parts of crude oil, 40 parts of water together with most of the ash separate within a few minutes. The separation of ash is completed by subsequently rinsing with about 150 to 200 parts of water, while continuously kneading. About 210 parts of a paste of coal and oil are produced containing only 1 40 per cent. of ash and 5 per cent. of water.

(5) A lignite containing 12.8 per cent. of ash and in the wet state in which it comes from the mine is ground in a suitable grinding device. In a known kneading machine, for instance in a Werner-Pfleiderer kneading apparatus, the ground coal is first mixed with water and made into a paste and subsequently kneaded with an equal weight of a lignite tar oil, calculated upon the dry coal, while adding 1 per cent. of sulfuric acid. After some minutes the water and most of the ash separate. There is produced a dispersion of coal and oil containing only 1 per cent. of ash. 50

(6) A coal containing 7.3 per cent. of ash is finely ground in an oscillating device with an equal weight of water. In a Werner-Pfleiderer kneading machine the coal is kneaded in the form of an aqueous paste with an equal weight of coal tar oil, calculated upon the dry coal, while adding 0.5 per cent. of caustic soda solution of 40° Bé. After some minutes the water and most of the ash separate. The dispersion of coal and oil of 50 per cent. strength produced has an ash content of 0.9 per cent.

(7) A coal containing 11.8 per cent. of ash is finely ground with an equal quantity of water in a suitable grinding apparatus. The coal is kneaded in a Werner-Pfleiderer kneading apparatus in the form of an aqueous paste with two thirds of its weight (calculated upon the dry coal) of coal tar oil, with the addition of 0.2 per cent. of caustic soda solution of 100 per cent. strength. After a short time most of the water together with the ash can be separated. The dispersion of coal and oil, thus already freed from 70 75

ash to a large extent, is then further kneaded in a Werner-Pfleiderer kneading apparatus in the presence of water and together with 2 per cent. of sulfuric acid calculated upon the weight of 5 coal. During the treatment a further quantity of ash separates together with the water. After the remaining free sulfuric acid has been neutralized with caustic soda solution there is obtained a dispersion of coal and oil freed from ash to a 10 very large extent.

(8) 100 parts of a ground lignite in the wet state in which it comes from the mine and containing 55 per cent. of water and 12.7 per cent. of ash, calculated upon anhydrous lignite, are 15 kneaded together with 18 parts of water so as to form a paste. On addition of 2 per cent. of sulfuric acid, calculated upon the dry lignite, and 45 parts of lignite tar oil, about 45 parts of water and a large part of ash are separated. 15 parts of 20 water are added to the paste of lignite and oil and kneading is continued. By kneading with this small quantity of water the residual ash is separated from the paste of lignite and oil and may be removed with the water. This procedure 25 is repeated four times more, using 15 parts of water each time. After the five treatments, the removal of ash has proceeded to such an extent that on further kneading the paste with water the supernatant rinsing water remains clear. 30 The paste of lignite and oil which is produced has an ash content of only 1 per cent. and a water content of about 20 per cent. that is to say, the water content of the lignite in the wet state as it comes from the mine has been reduced by about 35 50 per cent.

(9) 156 parts of a lignite in the wet state in which it comes from the mine and containing 55 per cent. of water, corresponding to 70 parts of dry lignite, are made into a paste in a suitable 40 kneading apparatus together with 44 parts of water and 5.3 parts of hydrochloric acid of 100 per cent. strength, and the paste is kneaded with about 63 parts of a lignite tar. After a short time about 70 parts of water separate, together with 45 most of the ash. By kneading in the presence of further 100 to 150 parts of water the separation of ash is finished. The dispersion of lignite and oil which is produced contains about 1 per cent. of ash and can be readily formed into 50 briquettes in the known briquetting plants.

(10) A coal containing 11.6 per cent. of ash is finely ground in an oscillating device with about an equal weight of water. The aqueous paste of coal is mixed in a suitable mixing apparatus with about an equal weight of coal tar oil, calculated upon dry coal, while adding 0.5 per cent. of caustic soda solution of 40° Bé., likewise calculated upon dry coal. The mixture is then introduced 6 times successively into a two- 55 roller mill during which operation the water and most of the ash separate. The dispersion of coal and oil obtained, of 50 per cent. strength, has an ash content of only 1 per cent.

(11) 150 parts of an aqueous coal paste which 60 consists of 60 parts of water and 90 parts of ground dry coal having an ash content of 11.5 per cent. are kneaded in a roller mill together with 0.5 per cent. of caustic soda solution, calculated upon the anhydrous coal and 70 parts of a coal tar oil. After the paste has passed through the rollers several times, about 54 parts of water and most of the ash separate from the hydrous, spongy mixture of coal and oil. The separation of ash is completed by subsequently rinsing with 75 a small quantity of water. In order to obtain a

dispersion of coal and oil which is easily conveyed further 10 parts of coal tar oil are rolled into the mixture. There is obtained a dispersion of coal and oil containing 1 per cent. of ash and about 3 per cent. of water.

(12) 128 parts of an aqueous paste of lignite consisting of 100 parts of ground lignite in the wet state in which it comes from the mine and having a water content of 55 per cent., 28 parts of water and 45 parts of dry coal having an ash 10 content of 15 per cent. are kneaded in a roller mill together with 2 parts of concentrated sulfuric acid and 45 parts of a lignite tar oil, calculated upon the dry coal. After the mixture has passed through the rollers several times, about 15 75 parts of water and most of the ash separate from the spongy dispersion of coal and oil. The separation is finished by rinsing the dispersion with a small quantity of water. There is obtained a paste of coal and oil which has a water content 20 of 8 per cent. and an ash content of about 1 per cent.

(13) 156 parts of a salt-containing crude lignite having a water content of 50 per cent. and corresponding to 78 parts of dry lignite are previously dried by waste heat to produce 120 parts of lignite having a water content of 35 per cent. The lignite is then made into a paste in a suitable kneading device together with 47 parts of water and 5.85 parts of hydrochloric acid of 100 per 30 cent. strength (7.5 per cent. calculated upon dry lignite) and the paste is kneaded with 44 parts of lignite hydrogenation oil. After a short time phase reversal occurs. About 45 parts of water and most of the ash separate. By kneading in 35 the presence of further 100 parts of water the separation of ash is completed. The paste of coal and oil is then further kneaded together with 51 parts of lignite hydrogenation oil. There is produced a paste of lignite and oil which has a water 40 content of about 10 per cent. and an ash content of about 1 per cent. It can be pumped at a temperature between 70° C. and 100° C.

We claim:

1. Process of preparing dispersions of coal and oil which comprises subjecting a paste of coal and water with oil while continuously maintaining the plastic condition to a squeezing and shearing action for a sufficient time to replace the water by the oil and materially reduce the ash content of 45 the coal and removing the ash and water which 50 separate.

2. Process of preparing dispersions of coal and oil which comprises subjecting a paste of coal and water with about an equal quantity of oil, calculated upon the dry coal, while continuously maintaining the plastic condition to a squeezing and shearing action for a sufficient time to replace the water by the oil and materially reduce the ash content of the coal and removing the ash and 55 water which separate.

3. Process of preparing dispersions of coal and oil which comprises kneading a paste of coal and water with oil by means of a roller mill wherein the oil is added by degrees while continuously 60 maintaining the plastic condition for a sufficient time to replace the water by the oil and materially reduce the ash content of the coal and removing the ash and water which separate.

4. Process of preparing dispersions of coal and oil which comprises kneading a paste of coal and water with about an equal quantity of oil, calculated upon the dry coal, by means of a roller mill wherein the oil is added by degrees while continuously 65 maintaining the plastic condition for a 70

75

sufficient time to replace the water by the oil and materially reduce the ash content of the coal and removing the ash and water which separate.

5. Process of preparing dispersions of coal and oil which comprises subjecting a paste of lignite containing not more than about 35 per cent. of water and water with oil while continuously maintaining the plastic condition to a squeezing and shearing action for a sufficient time to replace the water by the oil and materially reduce the ash content of the coal and removing the ash and water which separate.

6. Process of preparing dispersions of coal and oil which comprises subjecting a paste of lignite in the wet state in which it comes from the mine and water with oil while continuously maintaining the plastic condition to a squeezing and shearing action for a sufficient time to replace the water by the oil and materially reduce the ash content of the coal and removing the ash and water which separate.

7. Process of preparing dispersions of coal and oil which comprises subjecting a paste of coal and water with oil while continuously maintaining the plastic condition to a squeezing and shearing action for a sufficient time to replace the water by the oil and materially reduce the ash content of the coal, washing the dispersion with water during the kneading process and removing the ash and water which separate.

8. Process of preparing dispersions of coal and oil which comprises kneading a paste of coal and water with about an equal quantity of oil, calculated upon the dry coal, by means of a roller mill wherein the oil is added by degrees while continuously maintaining the plastic condition for a sufficient time to replace the water by the oil and materially reduce the ash content of the coal, washing the dispersion with water during the kneading process and removing the ash and water which separate.

9. Process of preparing dispersions of coal and oil which comprises subjecting a paste of coal and water containing a small quantity of an acid with oil while continuously maintaining the plastic condition to a squeezing and shearing action for

a sufficient time to replace the water by the oil and materially reduce the ash content of the coal and removing the ash and water which separate.

10. Process of preparing dispersions of coal and oil which comprises kneading a paste of coal and water, containing a small quantity of an acid, with oil by means of a roller mill wherein the oil is added by degrees while continuously maintaining the plastic condition for a sufficient time to replace the water by the oil and materially reduce the ash content of the coal and removing the ash and water which separate.

11. Process of preparing dispersions of coal and oil which comprises subjecting a paste of coal and water, containing a small quantity of a base, with coal tar oil while continuously maintaining the plastic condition to a squeezing and shearing action for a sufficient time to replace the water by the oil and materially reduce the ash content of the coal and removing the ash and water which separate.

12. Process of preparing dispersions of coal and oil which comprises kneading a paste of coal and water, containing a small quantity of a base, with coal tar oil by means of a roller mill wherein the oil is added by degrees while continuously maintaining the plastic condition for a sufficient time to replace the water by the oil and materially reduce the ash content of the coal and removing the ash and water which separate.

13. Process of preparing dispersions of lignite and oil which comprises kneading by means of a roller mill a paste of lignite and water with about an equal quantity of oil, calculated upon the dry lignite, said paste containing a small quantity of hydrochloric acid while continuously maintaining the plastic condition for a sufficient time to replace the water by the oil and materially reduce the ash content of the coal, washing the dispersion with water during the kneading process and removing the ash and water which separate.

SIEGFRIED KIESSKALT.  
HANS TAMPKE.  
KARL WINNACKER.  
ERNST WEINGAERTNER.